# EUROPEAN PATENT SPECIFICATION

(11) **EP 0 388 459 B1**
(45) Date of publication and mention of the grant of the patent: **29.11.1995**
(21) Application number: 89910628.0
(22) Date of filing: 27.09.1989
(51) Int. Cl.: F26B 3/04

(54) **PROCESS FOR DRYING WOOD**
VERFAHREN ZUM TROCKNEN VON HOLZ
PROCEDE POUR SECHER DU BOIS

(30) Priority: 27.09.1988 FI 884428
(43) Date of publication of application: 26.09.1990
(73) Proprietor: VALMET PAPER MACHINERY INC., 00620 Helsinki (FI)
(72) Inventor: SALIN, Jarl-Gunnar, SF-02210 Esbo (FI)
(74) Representative: Bayliss, Geoffrey Cyril
(86) International application number: FI8900186
(87) International publication number: WO9003543

(56) References cited:
- AT-B- 0 335 918
- DE-A- 1 729 259

## Description

The present invention relates to a process for drying wood in a drying tunnel through which the wood is gradually fed and there permeated by drying air which flows in the longitudinal direction of the tunnel. In particular, the present invention relates to such a process in which the drying tunnel is divided into two sections separated by an intervening space and with the drying medium divided into two circulating substreams. By means of the process improved quality of the dried wood is obtained with unchanged drying time or, alternatively, a shorter drying time with unchanged quality level.

Sawn wood should be dried to a moisture content of approx. 15-22 %, calculated on the dry weight of the wood, in order that the wood can be stored without biological attack in the form of mould etc. For drying wood at sawmills two main types of drying kiln are employed, so-called compartment kilns and progressive kilns (tunnel kilns), whereas timber-yard drying has practically ceased.

In the compartment kiln the entire quantity of wood which is to be dried is loaded into the kiln at one time, stacked in piles in known fashion. In principle any drying schedule whatsoever can be achieved in a kiln of this type. By drying schedule is meant how the temperature and moisture content of the drying air and its speed of flow through the wood pile are caused to vary during the drying period. It is therefore possible in this type of kiln to employ what is, by some criterium, the optimum drying schedule. This is the principal advantage of this kiln. The disadvantages include a relatively high energy consumption and that these kilns cannot be made especially large because otherwise the drying climate would vary too much in different parts of the wood load.

AT 335918 describes a wood drying process which employs a batch drier or series of batch driers. In each drier air is circulated in 2 streams which flow in opposite directions but all the wood enters the drier at the same time, is dried for the same length of time and removed at the same time.

In a conventional single-stage progressive kiln the piles of wood move gradually through the tunnel while new piles are loaded at regular intervals and at the same time dried piles are taken out from the other end of the tunnel. The drying air flows along the length of the tunnel in a counter-current direction through the piles. As the drying air flows through the piles it is cooled at the same time as its moisture content rises. Once the condition of the drying air which is fed into the tunnel and its speed have been chosen the changes in the temperature and moisture content of the air (i.e. the drying schedule) can no longer be controlled but depend only on the interaction with the wood through which the air flows. Thus unlike the compartment kiln, in a single-stage progressive kiln it is not possible to achieve any optimum drying schedule. Against this the progressive kiln has the advantage that the energy consumption is appreciably lower since the air which leaves the kiln is almost saturated and also heat recovery can readily be obtained. Further, the progressive kiln can advantageously be constructed for high capacities, 10,000 - 20,000 m³/annum.

A division of the progressive kiln into two stages has been proposed and has also come into use at some sawmills. In such a two-stage kiln the drying air is introduced into the tunnel between the stages so that part flows in a counter-current direction in the first stage of the kiln and part in a concurrent direction in the second drying stage. DE 1729259 describes this type of kiln. Compared with the single-stage progressive kiln, this two-stage progressive kiln has advantages primarily in regard to control technology as it has a number of self-regulating properties.

In the choice of the drying schedule for a compartment kiln or of the condition of the inlet air for a progressive kiln there are two main requirements which should be satisfied. On the one hand the final moisture content of the wood after the desired drying time should be that which is aimed for, and on the other hand the quality loss of the wood in drying should be as little as possible or at least acceptable. In general the speed of drying increases as the difference between the dry-bulb and wet-bulb temperatures of the air increases. The magnitude of the change in the quality of the wood is a more complicated function of the drying procedure, but roughly it can be said that the faster drying is carried out the greater are the quality losses. Thus in general it is a question of a compromise between slow drying with low throughput but good quality and fast drying with reduced quality. The compartment kiln has thereby achieved an increased importance for drying with preservation of quality since in such a kiln the drying schedule can be chosen in an optimum fashion. Drying can namely be carried out relatively fast without accentuating the quality loss.

Against the background of the aforesaid circumstances there has been a clear effort to try to construct progressive kilns with the characteristic advantages of this type but so that the disadvantage of the non-optimum drying schedule can be circumvented.

The quality loss of the wood in drying can be divided into two main components. One is that with high temperature levels and/or long drying times there is a flow of resin at knots etc. together with a darkening of the surface of the wood, the other is the occurrence of cracks in the wood. Of these two groups crack formation is, especially with thicker dimensions, clearly the more important. The cause of crack formation can be explained in the following manner. In drying the surface of the timber dries faster than the inner parts of the piece of timber because of the resistance to the movement of moisture within the material. When the fibre saturation point is reached, i.e. when the free water has been removed and only water bound to the wood substance remains, the wood starts to shrink. This means that an internal mechanical tensile stress arises in the surface of the timber. This tensile stress produced by shrinkage is balanced by a corresponding compressive stress in the inner parts of the timber. If the tensile stress in the surface layer exceeds the strength of the wood a rupture takes place, i.e. surface cracking occurs. Thus it is clear that if the difference in moisture content between the surface of the timber and its inner parts (the moisture profile) is pronounced the risk of crack formation increases, i.e. in rapid drying the risk increases. The matter is complicated, however, by the fact that wood is not a purely elastic material but exhibits viscoelastic properties. This means e.g. that if the surface of the timber is subjected for a longer time to tensile stress then creep occurs, i.e. there is a permanent extension of the surface layer. When drying has progressed so far that also the inner parts have reached the fibre saturation point, the surface has accordingly extended more than the inside and stress pattern is then reversed so that the outside is subjected to compressive stress and the inner parts to tensile stress. Hence during this latter phase of drying internal cracking of the timber can occur. Though these internal cracks cannot be seen they are of great importance in possible subsequent working of the timber.

Even though both the mechanisms of quality loss described above and the mechanisms of moisture transport have long been known at a qualitative level, the development of improved drying schedules has been almost exclusively empirical, i.e. based on direct experience concerning the final moisture content and quality which is obtained with the drying schedule which is tested. It can also be stated that the continuous measurement of the moisture content and profile of the timber during drying is admittedly possible but in practice very troublesome. On the other hand so far there exists no reliable method for the continuous measurement of the stress conditions in the timber or even for registration of when cracks occur.

It has, however, now proved possible with the aid of physical and mathematical methods of calculation to predict in a reliable fashion on the one hand how the moisture content and moisture profile of the timber develops and varies in different drying climates, and on the other to predict on the basis of these profiles what stresses occur and thus the risk of crack formation. Similarly there are possibilities to estimate resin flow and the colour change of the timber surface. Thus the final moisture content of the timber with a given drying schedule can be calculated and also the quality loss can be predicted with such models. Figure 1 may be cited as an example. In the figure the measured loss of value in per cent is marked on the vertical axis for quality grades 1-3 of 75 x 150 mm redwood timbers with various drying schedules. The horizontal axis shows an index calculated for the respective drying schedules which sets the maximum tensile stress in relation to the strength of the wood. Taking account of the experimental difficulties of such tests the correlation must be considered as entirely satisfactory.

When a conventional single-stage progressive kiln is analyzed with the aid of model calculations of this kind one obtains a picture which can be exemplified with the aid of Figure 2. The upper part of the figure shows on the vertical axis how the relative tensile stress in a 75 x 200 mm redwood timber changes as a function of the drying time expressed in days when the timber is dried from the fresh state down to a final moisture content of 19 % in 6 days under normal conditions. The lower part of the figure shows how the psychrometric difference (the difference between the dry-bulb and wet-bulb temperatures) varies in the wood pile when the drying air flows countercurrent through the timber with a speed of 4 m/s. From the figure it can be stated that no stress occurs in the wood during the first 24 hours since then the surface of the wood has not yet dried to below the fibre saturation point. After that the stress rises rapidly to reach its maximum towards the end of the second day. The stress then decreases continuously during the entire remaining drying time.

Since it is the maximum stress level which determines the risk of cracking (Figure 1), it can be seen that it is the psychrometric difference around the end of the second day that determines the quality loss of the wood. Both before and after this critical period the psychrometric difference could be greater than the levels given in Figure 2. This, however, can naturally not be changed in a conventional progressive kiln.

It has now unexpectedly been discovered that these negative properties associated with the conventional progressive kiln can to a large extent be eliminated if the kiln is divided into two drying stages in an appropriate fashion.

The principal characteristics of the invention are apparent from the accompanying Claim 1.

The present invention is accordingly based on the discovery that if the direction of flow of the drying air during the first stage of drying is countercurrent and during the latter stage is concurrent in relation to the wood, then a low psychrometric difference is obtained during the period which is critical for the quality of the wood with a increasing psychrometic difference on either side of this point. As an example of an embodiment of the invention Figure 3 is presented. By the reversed direction of flow of the drying air during the first stage, the psychrometric difference here decreases with time, which leads to a rapid drying at in the beginning, so that the fibre saturation point is reached already after 12 hours, whereas the stress level does not now rise as high as in Figure 2. During the second drying stage the conditions differ from those in a conventional kiln only in that the speed of the drying air can now advantageously be kept somewhat lower (for example 2.6 m/s) which gives a milder drying atmosphere during the critical period. The external conditions are unchanged both in the example concerning a conventional kiln (Figure 2) and in the example concerning the two-stage drying in accordance with the invention, so that a direct comparison is possible. One then sees that the high stress peak in Figure 2 has now been divided into two lower peaks. In the example in Figure 3 the dividing point between the two stages and also the temperatures and speeds of the drying air have been chosen so that these two stress peaks are of equal height and on as low a level as possible. This is achieved if the first drying stage represents approx. 1/3 and the second stage correspondingly 2/3 of the entire drying time (length of the drying tunnel). Further, the speed of the drying air in the first stage is advantageously kept somewhat higher and that in the second stage somewhat lower than that which is normal in a conventional single-stage progressive kiln. The stress peaks in Figure 3 are at an approx. 20 % lower level than the stress peaks in Figure 2 which leads to an appreciable reduction of the quality losses during drying (Figure 1) without the drying time (capacity) being changed. Alternatively this improvement obtained by means of the invention can be utilized so that the quality of the wood is kept unchanged but the drying time is shortened.

It may be noted that in the two-stage progressive kiln which was presented earlier the direction of flow of the drying air in relation to the wood is countercurrent in the first stage and concurrent in the second, which naturally has the consequence that the psychrometric difference is greatest in the neighbourhood of the critical drying period. With regard to the directions of flow this earlier design thus constitutes the worst imaginable alternative.

It has now also unexpectedly been discovered that, although drying in accordance with the invention is divided into two stages, important process units can be made common to both stages which appreciably simplifies the construction of the drying kiln without practically any effect on the quality-preserving properties of the invention. The kind of process units that can be made common are the heating unit for the drying air, fans for transport of the air through the timber, and the ventilation unit for maintenance of the desired air humidity.

As was apparent from Figure 3 it is advantageous to maintain a higher air speed in the first stage than in the second drying stage. Since, however, the number of timber piles in the first stage (tunnel length) is less than in the second stage this means that the flow losses are almost equal in the two stages despite the different speeds. Accordingly the air circulation in the two stages can be maintained by a single fan unit without the division of the air between the two stages departing significantly from that desired. Similarly it is apparent from Figure 3 that the air flows which are led into each of one of the drying stages at the ends of the tunnel do not differ very much as to their condition. This shows that the quality advantages of the invention can be retained even if air with the same condition, i.e. from the same heating unit, is fed into both the drying stages.

Figure 4 shows an example comparable with Figures 2 and 3 and in which the same air (psychrometric difference 9.5°C) is fed into both drying stages and in which the air speeds (3.12 and 2.24 m/s respectively) are matched so that the pressure drops are the same, i.e. a situation which can be obtained using only a single common heating unit and a single fan unit. It is apparent from the figure that the stress peaks are practically identical with the peaks in Figure 3. Further it is found that the drying air from each of the stages has almost the same condition (psychrometric difference approx. 4°C). Thus it is of no major consequence for the energy consumption whether the exhaust of moist air from the kiln takes place from the fist or the second stage or after mixing of the air from these stages, i.e. a common unit for exhaust of moist air and input of fresh air can be employed. An embodiment of the invention represented by Figure 4 shows that this two-stage drying tunnel is not to a decisive degree more complicated in its construction than a corresponding single-stage conventional drying tunnel but with the difference that the quality of the dried wood is considerably better despite an unchanged drying time. Alternatively the drying time can be appreciably shortened without changing the quality compared with a single-stage drying tunnel.

An example of an embodiment of the invention is illustrated in Figure 5, which shows a horizontal view in cross-section of an arrangement for implementation of the present process. In the figure wood pile 1 is waiting to be inserted into the drying tunnel through inlet door 2. Wood pile 3 in the first drying section is permeated by drying air flowing in a concurrent direction from return tunnel 4. Wood pile 5 in the second drying section is permeated by drying air flowing in a countercurrent direction from return tunnel 6. After the second section a dried pile of wood 7 is taken out through outlet door 8. After the respective drying sections the drying air is sucked out from the intervening space 9 with the aid of fan unit 10 to the conditioning unit. In order to maintain the desired moisture content of the drying air a portion of the drying air is sucked out through duct 11 and replacec with fresh air through duct 12. Part of the heat content in the exhaust air is recovered to the replacement air in heat exchanger 13. The drying air is heated to the desired temperature in hot-water or steam heated air heater 14 and is then conducted to said return tunnels 4 and 6. After the drying has progressed sufficiently said doors 2 and 8 are opened and a wood pile 5 is taken out to position 7 after which the entire row of wood piles 3 and 5 is moved a step forward and a new wood pile is inserted from position 1 into the first drying section after which the doors are closed and the drying process continued.

The process of the invention can also easily be supplemented by addition of a relaxation stage between the actual drying stages. If the wood, after passing through the first stage but before being fed into the second drying stage, is stored in essentially stationary air of approximately the same temperature as in the drying stage for a period of e.g. a few hours, a rapid equalization of the moisture profile of the wood in the thickness direction takes place. Upon entry into the second drying stage because of the increased moisture content in the surface layer more rapid drying is obtained, whereby the total drying time is not affected to a decisive degree despite the dead time which the relaxation stage represents. It is, however, earlier known that the visco-elastic properties (creep) of wood are accentuated by moisture changes. Because of these so-called mechano-sorptive effects the relaxation stage has a positive effect with respect to the development of stresses in the second drying stage. This can be exploited in the form of improved quality of the wood after drying or alternatively higher kiln capacity.

## Claims

1. A process of drying piles of wood in a drying tunnel having a first section adjacent to the inlet of the tunnel and a second longer section adjacent to the outlet, the timber piles being fed forward through each of said sections in a plurality of steps, such that a new pile of wood may be inserted into the tunnel each time the piles in the tunnel are moved forward a step, while being permeated by a gaseous drying medium transported primarily in the longitudinal direction of the tunnel, said drying medium being divided into two circulating substreams, characterised in that one of said substreams is caused to flow through the first section of the tunnel in the direction of motion of the piles of wood so that said one substream initially contacts the pile of wood last fed into the tunnel and thereafter successively piles of wood that have dried a longer period, and the other is caused to flow through the second section of the tunnel counter to the direction of motion of the piles of wood so that said other substream initially contacts a pile of wood that has been dried the longest period and thereafter successively piles of wood that have dried a shorter period; that the speed of the drying medium passing through the first section is higher than the speed of the drying medium passing through the second section; that when the piles of wood reach the juncture of the sections where the drying medium streams meet there is a relatively low psychrometric difference compared to the increasing psychrometric differences on either side of this juncture; and that said substreams are thereafter conditioned and recirculated.

2. A process according to claim 1, characterised in that said substreams after contact with the piles of wood are mixed and thereafter again divided into substreams which are conditioned and returned to their respective sections.

3. A process according to claim 1, characterised in that said substreams after contact with the piles of wood are mixed and conditioned and thereafter again divided into two substreams which are returned to their respective sections.

4. A process according to any of the preceding claims, characterised in that the length of the first drying section constitutes 25-50%, advantageously approx. 1/3, of the effective length of the entire drying tunnel.

5. A process according to any of the preceding claims, characterised in that the piles of wood after the first section but before the second section pass through a relaxation phase during which the piles of wood are surrounded by essentially stationary air with a condition essentially on the same level as in the actual drying sections.

6. A process according to any of the preceding claims, characterised in that the circulation of the drying medium is achieved by an organ which is common to both sections.

## Patentansprüche

1. Verfahren zum Trocknen von Holzstapeln in einem Trockentunnel, der einen ersten Abschnitt, benachbart zum Tunneleingang, und einen zweiten längeren Abschnitt, benachbart zum Tunnelausgang aufweist, wobei die Holzstapel durch jeden der Abschnitte in einer Vielzahl von Schritten vorwärts geführt werden, so daß bei Einführung eines neuen Holzstapels in den Tunnel jeweils die Stapel im Tunnel einen Schritt vorwärts bewegt werden, während ein gasförmiges Trockenmedium durch sie hindurchgeht, das primär in Längsrichtung des Tunnels geführt wird, wobei das Trockenmedium in zwei zirkulierende Teilströme unterteilt wird, dadurch gekennzeichnet, daß einer der Teilströme durch den ersten Abschnitt des Tunnels in Bewegungsrichtung der Holzstapel geführt wird, so daß der eine Teilstrom anfangs mit dem Holzstapel in Kontakt kommt, das zuletzt in den Tunnel eingeführt wird, und danach nacheinander mit den Holzstapeln, die einen längeren Zeitraum getrocknet worden sind, und der andere durch den zweiten Abschnitt des Tunnels entgegengesetzt zur Bewegungsrichtung der Holzstapel geführt wird, so daß der andere Teilstrom anfänglich mit den Holzstapeln in Kontakt kommt, die den längsten Zeitraum getrocknet worden sind, und danach nacheinander mit den Holzstapeln, die einen kürzeren Zeitraum getrocknet worden sind; daß die Geschwindigkeit des Trockenmediums, das durch den ersten Abschnitt geführt wird, höher ist als die Geschwindigkeit des Trockenmediums, das durch den zweiten Abschnitt geführt wird; daß, wenn die Holzstapel den Verbindungspunkt der Abschnitte erreichen, wo sich die Trockenströme treffen, ein relativ niedriger Feuchtigkeitsunterschied besteht im Vergleich mit den erhöhten Feuchtigkeitsunterschieden auf beiden Seiten dieses Verbindungspunktes; und daß die Teilströme danach auf Normalfeuchtigkeit gebracht und rezirkuliert werden.

2. Verfahren nach Anspruch 1, dadurch gekennzeichnet, daß die Teilströme nach dem Kontakt mit den Holzstapeln vermischt und danach wiederum in Teilströme aufgeteilt werden, die auf Normalfeuchtigkeit gebracht und in ihre entsprechenden Abschnitte zurückgeführt werden.

3. Verfahren nach Anspruch 1, dadurch gekennzeichnet, daß die Teilströme nach Kontakt mit den Holzstapeln vermischt und auf Normalfeuchtigkeit gebracht und danach wiederum in zwei Teilströme aufgeteilt werden, die in ihre entsprechenden Abschnitte zurückgeführt werden.

4. Verfahren nach einem der vorangegangenen Ansprüche, dadurch gekennzeichnet, daß die Länge des ersten Trocknungsabschnittes 25 bis 50 % einnimmt, vorzugsweise etwa ¹/₃ der effektiven Länge des gesamten Trockentunnels.

5. Verfahren nach einem der vorangegangenen Ansprüche, dadurch gekennzeichnet, daß die Holzstapel nach dem ersten Abschnitt jedoch vor dem zweiten Abschnitt eine Beruhigungsphase durchlaufen, bei der die Holzstapel von im wesentlichen stehender Luft mit einem Feuchtigkeitsgehalt umgeben sind, der im wesentlichen dem in dem gegenwärtigen Abschnitt entspricht.

6. Verfahren nach einem der vorangegangenen Ansprüche, dadurch gekennzeichnet, daß die Zirkulation des Trockenmediums mit einer beiden Abschnitten gemeinsamen Einrichtung erfolgt.

## Revendications

1. Un procédé de séchage de piles de bois dans un tunnel séchant, ayant une première section adjacente à l'entrée du tunnel et une seconde section plus longue adjacente à la sortie, les piles de bois d'oeuvre étant envoyées à travers chacune desdites sections en plusieurs étapes, de façon à ce qu'une nouvelle pile de bois puisse être insérée dans le tunnel chaque fois que les piles dans le tunnel sont déplacées vers l'avant graduellement, pendant qu'elles sont imprégnées par un moyen séchant gazeux transporté en premier lieu dans la direction longitudinale du tunnel, ledit moyen séchant étant réparti en deux sous-courants circulants, caractérisés en ce qu'un desdits courants secondaires est amené à s 'écouler à travers la première section du tunnel dans la direction du mouvement des piles de bois de sorte que ledit sous-courant initialement entre en contact avec la pile de bois la dernière entrée dans le tunnel et ensuite successivement avec les piles de bois qui ont séché pendant une plus longue période, et l'autre est amené à s'écouler à travers la seconde section du tunnel en sens inverse de la direction de mouvement des piles de bois de sorte que ledit autre sous-courant initialement entre en contact avec une pile de bois qui a été séchée pendant la plus longue période et ensuite successivement avec les piles de bois qui ont séché pendant une période plus courte; que la vitesse du moyen de séchage passant à travers la première section est plus élevée que la vitesse du moyen de séchage passant à travers la seconde section; que lorsque les piles de bois atteignent la jonction des sections où les courants de moyen de séchage se rencontrent, il y a une différence psychrométrique relativement basse comparée aux différences psychrométriques croissantes sur chaque côté de cette jonction; et que lesdits sous-courants sont ensuite traités et remis en circulation.

2. Un procédé selon la revendication 1, caractérisé en ce que lesdits sous-courants après contact avec les piles de bois sont mélangés et ensuite encore divisés en sous-courants qui sont traités et retournés à leurs sections respectives.

3. Un procédé selon la revendication 1, caractérisé en ce que lesdits sous-courants après contact avec les piles de bois sont mélangés et traités et ensuite encore divisés en deux sous-courants qui sont retournés à leurs sections respectives.

4. Un procédé selon l'une quelconque des revendications précédentes, caractérisé en ce que la longueur de la première section de séchage constitue 25-50%, avantageusement approximativement 1/3, de la longueur effective du tunnel de séchage entier.

5. Un procédé selon l'une quelconque des revendications précédentes, caractérisé en ce que les piles de bois après la première section mais avant la seconde section passent à travers une phase de relaxation durant laquelle les piles de bois sont entourées d'air essentiellement stationnaire avec un état essentiellement du même niveau que dans les sections de séchage effectives.

6. Un procédé selon l'une quelconque des revendications précédentes, caractérisé en ce que la circulation du moyen de séchage est réalisée par un organe qui est commun aux deux sections.
